

Aug. 1, 1972

KIMINARI KAWAKAMI ET AL

3,681,057

ALUMINUM KILLED-STEEL

Filed June 10, 1970

Fig. 3



Fig. 2



Fig. 1



KIMINARI KAWAKAMI AND  
SHIZUNAO YAMAGISHI

By

*Linton and Linton*  
ATTORNEYS

1

3,681,057

### ALUMINUM KILLED-STEEL

Kiminari Kawakami and Shizunao Yamagishi, Fukuyama, Japan, assignors to Nippon Kokan Kabushiki Kaisha, Tokyo, Japan

Filed June 10, 1970, Ser. No. 45,108

Claims priority, application Japan, June 12, 1969,  
44/45,748

Int. Cl. C22c 39/20

U.S. Cl. 75—124

1 Claim

### ABSTRACT OF THE DISCLOSURE

An Al-killed steel consisting of a Si-Al-Nb system that can be produced with a good yield and has excellent surface quality for providing a line pipe tensile strength of more than 60 kg./mm.<sup>2</sup>, good low temperature toughness and distinguished weldability.

The present invention is concerned with an aluminum killed-steel of excellent quality and more particularly to Al-killed steel of an improved composition.

In recent years the demands for line pipe that is used for the extended transportation of crude oil petroleum products, natural gas and the others has more and more increased, and the diameter of said pipe has increased. It is well known that a welded pipe, which is made of plate, is widely employed as said line pipe. The size and quality of these materials are specified in known API Standards, e.g. API-5LX-60, API-5LX-65, etc. In such steels, it is needless to say that the workability and weldability as well as the mechanical properties of said line pipe are required to be of high quality. Special attention should be paid to the low-temperature notch toughness of said steels, when services in the coldest regions are to be considered. It will be understood that the chemical composition of said API Standards is presently insufficient since these Standards may be tentative and leave room for development. It is well known that the composition of API x-series Standards shall conform to the chemical requirements agreed upon between the purchaser and manufacturer.

This invention has mechanical properties as specified in said API Standards. The features lie in the addition of low silicon, Sol. Al and higher content of Nb, without addition of costly V, Ti and the like.

An object of this invention is to provide an Al-killed steel having a high yield point of more than 65,000 p.s.i. that can be produced with ease and stability.

Another object of this invention is to provide an Al-killed steel having excellent toughness in low temperature services.

Other objects and advantages of the invention will be apparent from the following description and the accompanying drawing, in which

FIG. 1 is a histogram showing the surface quality of ordinary steel;

FIG. 2 is a histogram from cold ingot treatment; and

FIG. 3 is a histogram of the present invention ingot.

Steel of the present invention is produced as an Al-killed-steel. General, surface cracks of a slab, which is shaped from said Al-killed ingot, are observed. Such cracks are generated by the precipitation of AlN, which is formed by the cooling of the surface layer of the hot ingot. It is needless to say that said precipitation goes on as the track time becomes longer. According to many experiments, it has been discovered that said generation of cracks can be avoided by means of adding low Si, instead of cold ingot treatment that is cooled to room temperature and then charged into a soaking pit. That is, a

2

small content of Si is effective to prevent the ingot from precipitation of AlN at the cooling stage of said ingot.

The Si content of more than 0.15% has little effect on preventing the ingot from precipitation of AlN. When 5 the Si content is less than 0.02% the steel increases in inclusion and results in dirty steel. A lowering of yield will be inevitable.

The C content of the present invention is limited to a range from 0.13 to 0.23%. A C content of more than 0.13% is required in order that the tensile strength of more than 60 kg./mm.<sup>2</sup> is kept with stability. However, when the C content is above 0.23%, weldability of the steel will be lower. Such a steel is undesirable, because weldability of the steel is an important factor of the invention.

An Mn content of more than 1.5% makes weldability of the steel worse in connection with the C content. The tensile strength of the steel including the Mn content of less than 1.2% becomes insufficient in connection with 20 the C content. Accordingly, the range of the Mn content of the invention is from 1.2 to 1.5%.

Effects of Nb added to steel lie in the precipitation effect in ferrite grain and grain refining effect by Nb carbide. The best suited range of Nb content in the invention steel is from 0.01 to 0.05%. Even though more than 0.05% Nb was added, larger effects cannot be expected, because said effects amount to a saturated condition, and less than 0.01% Nb has no effect.

A Sol. Al content in the range from 0.02 to 0.05% 30 has the highest grain refining effect. Even though said content was above 0.05%, there is no said effect being in proportion to said content. When Sol. Al content is less than 0.02%, said grain refining effect cannot be expected.

Mechanical properties in a low temperature services, 35 e.g. low temperature notch toughness, are possible with the above mentioned grain refining effect of Nb carbide and Sol. Al content.

Number of steel: 4

40 Analysis of crude steel: as mentioned in Table 4  
Steel making furnace: basic oxygen furnace  
Ingot weight, slab size and plate dimension: as mentioned in Table 1

Mechanical properties: as mentioned in Table II

45 Merits of the invention steel, which is confirmed in the above experiments, are as follows:

(1) Cold ingot treatment does not need to be used. Accordingly, an increase in the capacity of soaking pit is 6 t./hr.

(2) There is little surface crack in the slab.  
(3) Cleanliness of ingot and low temperature toughness of steel are remarkably improved.

(4) Resistibility for hydrogen brittleness increases and white spot of slab and plate decreases.

(5) Defects that are apt to be generated at welded portions can be checked.

Each of the accompanying drawing figures is a histogram of the surface quality of slabs. Axis of abscissas in said figures shows the rate of reduction of weight, which is based on the repairing operation, with a rank. Said reduction of weight shown as numeral 1 is less than 0.5%, numeral 2 is from 0.5 to 0.1%, numeral 3 is from 1.0 to 2.0%, numeral 4 is from 2.0 to 2.5%, numeral 5 is more than 2.5% and numeral 0 is impossible to be repaired, which is scrapped.

According to the above histogram it will be understood that the surface quality of the invention is excellent in comparison with other prior steels.

70 This invention steel is possible to be widely utilized as structural materials, in addition to use as materials for line pipe.

TABLE I.—ANALYSIS OF CRUDE STEEL

| Comp.<br>steels | C              | Si   | Mn    | P     | S     | Nb    | Sol. Al                                              | Weight,<br>t. Slab size | Dimensions of plate                                                         |
|-----------------|----------------|------|-------|-------|-------|-------|------------------------------------------------------|-------------------------|-----------------------------------------------------------------------------|
| A.....          | 0.212          | 0.14 | 1.34  | 0.019 | 0.019 | 0.018 | { 0.039<br>0.040<br>0.026<br>0.028<br>0.033<br>0.032 | 23,000                  | 245 thickness x 1.600 width x 12.7 thickness x 3.308 width x 12.340 length. |
| B.....          | 0.206          | 0.15 | 1.35  | 0.017 | 0.022 | 0.019 | { 0.028<br>0.032                                     |                         |                                                                             |
| C.....          | 0.197          | 0.15 | 1.36  | 0.017 | 0.018 | 0.022 | { 0.030<br>0.028<br>0.020                            | 29,000                  | 205 thickness x 1.900 width x 12.1 thickness x 3.152 width x 12.340 length. |
| D.....          | 0.199          | 0.15 | 1.32  | 0.014 | 0.017 | 0.017 | { 0.032<br>0.026<br>0.020                            |                         |                                                                             |
| Invention.....  | { 0.13<br>0.23 | 0.15 | 1.20  | ..... | ..... | 0.010 | 0.020                                                |                         |                                                                             |
|                 | Less           | 1.50 | ..... | ..... | ..... | 0.050 | 0.050                                                |                         |                                                                             |

TABLE II.—MECHANICAL PROPERTIES

| Test value steels   | Yield<br>point,<br>kg./mm. <sup>2</sup> | Tensile<br>strength,<br>kg./mm. <sup>2</sup> | Elongation,<br>percent | Impact test                |    |
|---------------------|-----------------------------------------|----------------------------------------------|------------------------|----------------------------|----|
|                     |                                         |                                              |                        | value,<br>kg.-m.<br>EV-18* |    |
| A.....              | 46.7                                    | 62.8                                         | 34.0                   | 2.29                       | 20 |
|                     | 46.4                                    | 61.7                                         | 35.0                   | 2.22                       |    |
|                     | 45.7                                    | 61.9                                         | 29.0                   | 2.22                       |    |
| B.....              | 47.7                                    | 65.7                                         | 32.5                   | 2.39                       |    |
|                     | 48.0                                    | 63.6                                         | 32.0                   | 2.39                       |    |
|                     | 49.0                                    | 65.5                                         | 30.5                   | 2.36                       |    |
| C.....              | 45.9                                    | 62.8                                         | 31.8                   | 3.12                       | 25 |
|                     | 45.3                                    | 61.8                                         | 34.0                   | 3.41                       |    |
|                     | 44.7                                    | 61.8                                         | 36.0                   | 3.39                       |    |
| D.....              | 44.2                                    | 60.1                                         | 36.0                   | 3.19                       |    |
|                     | 43.3                                    | 60.2                                         | 38.0                   | 3.27                       |    |
|                     | 42.6                                    | 59.5                                         | 38.0                   | 3.08                       |    |
| Standard value..... | (1)                                     | (2)                                          | .....                  | 2.07                       |    |

<sup>1</sup> Than 43.<sup>2</sup> Than 55.

\*2 mm. V notch Sharpy test; test temperature -18° C.

15 We claim:

1. An Al-killed steel consisting of 0.13 to 0.23% C, 0.02 to 0.15% Si, 1.20 to 1.50% Mn, 0.02 to 0.05% Sol. Al, 0.01 to 0.05% Nb, and the balance being Fe and unavoidable impurities.

20

## References Cited

## UNITED STATES PATENTS

|           |         |          |        |
|-----------|---------|----------|--------|
| 3,562,028 | 2/1971  | Heitmann | 75—124 |
| 3,328,211 | 1/1967  | Nakamura | 75—124 |
| 3,554,734 | 1/1971  | Kikkawa  | 75—125 |
| 3,259,488 | 12/1967 | Nakamura | 75—124 |
| 3,357,822 | 7/1966  | Miyoshi  | 75—124 |

30 HYLAND BIZOT, Primary Examiner